

W. D. COOLIDGE.  
ELECTRICAL CONTACT.  
APPLICATION FILED DEC. 17, 1912.

1,089,907.

Patented Mar. 10, 1914.

Fig. 1.



Fig. 2.



Fig. 3.



Fig. 4.



Fig. 7.



Fig. 5.



Fig. 6.



Witnesses:

Benjamin B. Bruce  
Helen Oxford

Inventor:

William D. Coolidge,  
by Almon D. Davis  
His Attorney.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## ELECTRICAL CONTACT.

1,089,907.

Specification of Letters Patent. Patented Mar. 10, 1914.

Original application filed March 20, 1912, Serial No. 685,113. Divided and this application filed December 17, 1912. Serial No. 737,214.

To all whom it may concern:

Be it known that I, WILLIAM D. COOLIDGE, a citizen of the United States, residing at Schenectady, county of Schenectady, State of New York, have invented certain new and useful Improvements in Electrical Contacts, set forth in my application, Serial No. 685,113, filed March 20, 1912, of which this is a division.

My invention relates to electrical contacts, particularly for rheotomes or other vibratory circuit making and breaking devices, ordinarily used as sparking or igniting contacts for gas-engines, as circuit controllers for regulators, and for other like purposes. In apparatus of this character, vibratory contact terminals of expensive metals, such as platinum and iridium, have heretofore been used, and it was found that these contacts deteriorated and became destroyed, so as to be unfit for further use, within a comparatively short time. The contacts were found to blacken and pit; their contacting surfaces became deformed by the continuous hammering action and by the formation of irregular and variably distributed small protuberances due, probably, to the transference of material from the cathode to the anode, whereby the normal distance between the contacts was reduced and "bridges" were often formed between the two contacts. It was also found that the accidental wetting of the contacts with oil seriously interfered with their operation. In addition to this, the materials heretofore used for vibratory contacts are softened by the heat of the sparks passing between them, to such an extent as to cause welding, or incipient welding.

Vibratory contacts are largely used in regulators of the kind known as Tirrill regulators, and the use of platinum or iridium, or platinum-iridium, or silver, for the contacts, results in rendering the regulators operative within a comparatively short time, because these regulators depend for their successful operation upon the periodical complete making and breaking of a circuit or circuits by the contacts. The normal space

between the contacts is between 1/32 inch and 1/100 inch, and this space is reduced by the formation of protuberances on one or both contacting surfaces to such extent that the sparks between them are frequently maintained during the periods of the "breaks", so that no real break of circuit takes place, but only an irregular and insufficient increase of resistance. The deformation of the contact surfaces, due to the hammering action, has a like result, and all these variable deformations result in a variation of the number of points of actual physical contact, whereby the transition resistance is irregularly varied.

My invention is designed to overcome these difficulties and it consists broadly in make and break contacts of metallic tungsten, preferably in the wrought or malleable form.

It is a well-known fact that tungsten, when heated to redness in air, is soon covered with a layer of oxid which is practically an insulator, especially in the cold state, and this property of tungsten would seem to make this material unfit for use as contacts. But I have found by experiment that this is not so, and that by reason of the light powdery or flocculent condition of the oxid, the same is shaken off almost as quickly as it is formed, so that vibratory contacts of tungsten, and especially of wrought or malleable tungsten, can be used with great advantage.

I have found that the pitting of the contacts made of tungsten, while theoretically not absent, is practically insignificant; that the normal distance between the contacts remains sensibly constant during a long period; that no welding or incipient welding of the contacts occurs, and that the presence of oil on the contact surfaces does not interfere with their operation. In consequence of these properties of tungsten which I have ascertained by long continued experiments, contacts of this material have a very much longer life than contacts made of any other material known to me, or of any material that has heretofore been used.

In a comparative test, I have found that a pair of tungsten contacts, after having made thirty-two millions of makes and breaks, were still clean and symmetrical, and apparently as good as new; while a pair of platinum contacts operated under the same conditions and with the same number of makes and breaks, were found to have become so badly pitted, consumed and deformed as to be unfit for further use.

One of a pair of contacts is usually mounted on a resilient support, such as a spring, and the other to a rigid support, and the joinder between the contacts and supports should be very intimate so that the contacts will not become loose by the hammering action to which they are subjected. I secure this result either by fusing to one face of the tungsten contact a backing of a rather bulky piece of a metal of superior conductivity for heat and electricity, such as copper, silver or gold, and fasten the backing to a spring or rigid support by screws or other mechanical means; or I interpose the backing of superior conductivity between the contact and the support by fusion to both, that is to say, by using the backing as a solder. In either case, the heat generated in the contact is carried away rapidly. A new and improved process of thus joining tungsten contacts to their supports is hereinafter fully described, but no claim is herein made for the same, since that invention is claimed in my aforesaid original application Serial Number 685,113, filed March 20, 1912, of which this is a division.

Tungsten cannot be joined satisfactorily to other metals by soldering in the ordinary manner. This difficulty is apparently due to the ease with which a thin film of oxid forms on the surface of the tungsten. The soldering metal either will not stick or when apparent adhesion has been produced I find that when subjected to any strain the soldering metal breaks away as though the tungsten broke away from the film of oxid. The joinder of tungsten contacts or other bodies of tungsten to the backing of the metal of superior conductivity is, however, successfully accomplished by causing melted copper, silver or gold to flow over the tungsten surface in an atmosphere of hydrogen, as more specifically hereinafter set forth.

In the accompanying drawings, Figure 1 shows a form of mold suitable for holding the contacts during the process of heating in hydrogen; Fig. 2 shows the parts of a contact before attaching; Fig. 3 illustrates the completed contact; Fig. 4 illustrates an apparatus by which a tungsten contact is directly attached to a spring or other support; Fig. 5 illustrates another modification according to which a body of copper is cast directly into contact with a piece of tungsten; Fig. 6 shows a machined contact at-

tached to a support, and Fig. 7 illustrates co-  
porting rheotome or spark contacts.

In carrying out the process as above outlined, I find it highly desirable to completely remove from the surface of the tungsten body all the loosely adherent metal or oxid which I find is left by the preliminary process of shaping the tungsten. Unless this is done, I find that in some cases the tungsten may be torn away from its backing or support at this loosely adherent surface layer, part of which will be found clinging to the copper or other metal used as solder. In order to remove this surface layer I prefer to bring the body of tungsten into contact with melted nitrite of sodium or potassium for a few seconds or with hot caustic potash or caustic soda solution for a longer time. This leaves a perfectly bright surface of solid metal.

When it is desired to fasten a small disk of tungsten to a tack or support of steel, which may then be conveniently riveted or otherwise fastened to terminal supports, as shown in Fig. 7, the operation may be carried out as follows: The parts particularly used for building up the contact are shown in Fig. 2. An iron or steel tack is placed in a holder or mold 1 shown in Fig. 2, which may consist of graphite, magnesia, fire clay, alumina or other refractory material. As illustrated by a portion of the holder 1 broken away, the shank 2 of the tack is inserted in a hole so that the tack is supported by the shoulder 3 and centered by its shank. A plate of copper 4 is placed upon the tack, and disk 5 of tungsten is placed upon the copper, the three parts being thus properly held in position. The connecting channels 6 between the holes in the mold are provided for the purpose of allowing the circulation of hydrogen during the subsequent heating process. Only a few holes have been indicated but of course as many as desired may be used with a single holder. The holder with the parts of the contact thus assembled is then placed in a suitable furnace and heated in a hydrogen atmosphere to a temperature above the melting point of copper. A porcelain tube furnace, with hydrogen passed through the tube, is suitable for this purpose. Under these conditions in the absence of oxygen the copper will wet the surface of the tungsten so as to form a continuous metallic union between the tungsten and the steel. When removed from the furnace and allowed to cool the tungsten and steel will be found to be intimately united by a backing or layer of copper as indicated in Fig. 3.

In some cases, as when joining the tungsten contact directly to a steel spring, it is convenient to carry out the heating operation with an electric arc as shown in Fig. 4. In this case the spring 7 is held in a clamp

8, the metallic jaws 9 of which hold the spring and abstract heat from it so as to avoid drawing its temper during the heating operation. The jaws 9 may be tightened by the strap 10. The tungsten contact 11 is provided with a teat 12 which passes through a hole in the spring. A small body of copper such as the copper wire 13 is introduced in close proximity to the spring and tungsten contact. The spring and contact thus assembled are placed in a container 14 open at the bottom and supplied with a stream of hydrogen gas through a tube 15. An arc fed by a suitable source of current such as a battery 16, is then drawn between the teat 12 and the hand electrode 17, thereby heating the tungsten contact to the melting point of copper at which temperature the melted copper will be drawn into the contracted space under the tungsten disk by capillary forces. The copper in the presence of hydrogen wets the contiguous surfaces of tungsten and steel in the contracted space thereby making a continuous metallic junction between the contact and the spring. Of course, in the same manner that steel is joined to tungsten, other metals such as nickel, cobalt, platinum, molybdenum, or even another body of tungsten, may be joined to tungsten. When it is desired to attach tungsten to platinum, I prefer to use gold as the soldering metal.

According to a modified process a mass of copper is cast into contact with the tungsten. Ordinarily copper by reason of its dissolved gases or other impurities will not wet the surface of tungsten. Either the tungsten acts as a deoxidizer with respect to the copper and becomes coated with oxid or dissolved oxides of copper lower the surface tension of copper relatively to tungsten. I have found, however, that if the melted copper is treated previous to casting with a small quantity of an oxidizable boron material such as elemental boron, boron sub-oxid or boron carbide, which combines with the dissolved impurities, the copper will then wet and permanently adhere to the surface of the tungsten. This process of purifying copper is described in an application filed by E. Weintraub, Serial Number 636,270, filed June 30, 1911. Elemental boron and boron carbide are now well-known to chemists. Boron sub-oxid is the product of the reduction of boric anhydride with magnesium at a temperature of 1300° C. or higher. The reduction mass left after washing with dilute sulfuric acid is a brown powder. The treatment of the copper is carried out by adding 1/30 to 1/10 of 1% or more of boron or of a boron compound containing an equivalent amount of boron in the reduced state while the copper is heated considerably above its melting point, say 1200 to 1300° C. or higher. The copper

thus prepared is then cast into contact with the tungsten body which may for example be placed in the bottom of a magnesia or alumina crucible 18 as shown in Fig. 5. After cooling, the mass of copper and tungsten thus joined together is removed and the copper may be machined so as to attach it in any approved manner to electrical apparatus. Fig. 6 is illustrative of a contact made in this way, the copper 19 being attached by means of a screw 20 to the supporting part 21 indicated by dotted lines.

As a modification I may cause the purification and attachment of copper to the tungsten body to take place in one operation. This may be done by placing the disk of tungsten, for example, in the bottom of a crucible as shown in Fig. 5, placing the boron material upon the tungsten and then adding copper. The contents of the crucible are then heated to a temperature several hundred degrees in excess of the melting point of copper. The exclusion of air during the heating process is not essential although desirable.

According to another modification the copper is caused to unite metallically with a tungsten body by heating to a temperature considerably above its melting point in a vacuum preferably to a temperature about 1400° C. Under these conditions an oxid of tungsten cannot exist, the oxid at this temperature being dissociated into metallic tungsten and oxygen. The copper itself appears to lose at least part of its dissolved gases. The operation may be carried out by placing a body of tungsten and a quantity of copper in a crucible, as shown in Fig. 5, and heating the crucible and its contents in a vacuum furnace such as shown in Arsem Patent No. 785,535. After being heated to the required temperature the copper and tungsten are simply allowed to cool in contact with each other. Upon removal from the crucible, the copper may be machined. The tungsten terminal 22, Fig. 7, is attached to an armature 23, and cooperates with a stationary tungsten contact 24.

What I claim as new and desire to secure by Letters Patent of the United States, is:

1. An electrical make-and-break contact of tungsten.
2. An electrical make-and-break contact of malleable tungsten.
3. An electrical make-and-break contact of tungsten, and a backing for the same of a metal of superior electric and thermal conductivity intimately joined thereto.
4. An electrical make-and-break contact of tungsten integrally joined to a metal backing of superior electric and thermal conductivity.
5. An electrical make-and-break contact of tungsten, a support for the same and a contact backing of a metal of superior elec-

tric and thermal conductivity intervening between the contact and support and integrally joined to both.

6. An electrical vibratory make-and-break contact of tungsten.

7. An electrical make-and-break impact contact of tungsten.

In witness whereof, I have hereunto set my hand this 16th day of December, 1912.

WILLIAM D. COOLIDGE.

Witnesses:

HELEN ORFORD,

BENJAMIN B. HULL.